

106-18.18

SR

MTR49

XR

1,523,814

Search No. 1

Jan. 20, 1925.

1,523,814

W. G. LINDSAY

CROSS REFERENCE

FIREPROOF FABRIC AND PROCESS OF MAKING SAME

Filed Dec. 14, 1917

FIG 1

FIG 2



Inventor  
William G. Lindsay  
By His Attorneys  
Edwards, Sager & Dover

1523814  
OR IN 425/260

Patented Jan. 20, 1925.

1,523,814

# UNITED STATES PATENT OFFICE.

WILLIAM G. LINDSAY, OF NEWARK, NEW JERSEY, ASSIGNOR TO THE CELLULOID COMPANY, A CORPORATION OF NEW JERSEY.

## FIREPROOF FABRIC AND PROCESS OF MAKING SAME.

Application filed December 14, 1917. Serial No. 207,117.

To all whom it may concern:

Be it known that I, WILLIAM G. LINDSAY, a citizen of the United States, residing at Newark, in the county of Essex and State 5 of New Jersey, have invented certain new and useful Improvements in Fireproof Fabrics and Processes of Making Same, of which the following is a specification.

The principal object of my invention is to 10 provide a new and improved coated fireproof fabric for use in various places, and a method of preparing the same. This and other objects will be indicated in connection with the following specification, in which 15 I have disclosed one specific embodiment of my invention and the procedure in accordance therewith.

My improved coated fireproof fabric is especially adapted for use on airplane wings. 20 After the wing frames have been made, the cloth is ordinarily wrapped once around the frame, sleeve-like, and then coated with some varnish-like preparation. It is highly desirable that the fabric be fireproof, but 25 it is difficult to obtain this quality and at the same time get other desirable characteristics such as waterproofing, strength, flexibility, and a proper shrinkage of the fabric so as to draw it on the frame.

30 Nitrocellulose or pyroxylin makes a very good coating so far as flexibility and shrinking effect are concerned, but it is highly inflammable. By my invention herein disclosed, I have succeeded in devising a way 35 in which to use such a substance for coating as nitrocellulose and obtain these desirable qualities, but at the same time make the coated fabric fireproof as well as waterproof.

40 Attempts have been made to make a pyroxylin coating fireproof by mixing some fireproofing ingredient therewith, but such ingredient must be present in large proportion to effect the desired result, and when 45 it is present in this large proportion it detracts from the other desirable qualities of the nitrocellulose.

50 Stated in somewhat general terms, according to one aspect of my invention, it involves impregnating the fabric with a fireproofing substance and then coating it with a coating of reduced or low inflammability, whereby the resultant coated fabric will be effectively fireproof.

55 The product is shown in the accompany-

ing drawings, in which Figs. 1 and 2 are sections, the latter enlarged, of a fabric coated with the resultant composition.

My invention may be practiced in a variety of ways; I will now give one specific 60 example of procedure in accordance therewith. The fabric is first applied to the airplane frame and sewed in place, being drawn to such an ordinary degree of tightness as may be convenient for sewing. Of course, it should be made much tighter than this when ready for service. Next, a water solution of ammonium phosphate is applied with a brush thoroughly saturating the cloth. Then the treated cloth is allowed to 70 dry, leaving it impregnated with the ammonium-phosphate.

I prepare a solution of nitrocellulose and tricresylphosphate according to the following formula:

|                    | Parts. |
|--------------------|--------|
| Pyroxylin          | 100    |
| Tricresylphosphate | 50     |
| Acetone            | 300    |
| Methyl alcohol     | 600    |
| Amyl acetate       | 300    |

For the nitrocellulose I use a good soluble variety such as is ordinarily well-known to manufacturers of "celluloid." This pyroxylin solution is then applied with a brush and, after it dries, another coat may be applied if so desired and so on to any number of coats. In drying it shrinks the fabric so as to draw it tight on the frame; increases 85 its tensile strength, the coating unites intimately with the fabric so as to have a unitary character therewith, and leaves a smooth external surface giving a minimum of friction with the air.

In the drawings the fabric is indicated at A, the coating composition at B, C.

The dried ammonium phosphate will be in the form of crystals which will adhere to the fibres of the fabric and arrange themselves in irregular manner. The pyroxylin solution will penetrate into the crevices between the ammonium phosphate crystals and obviously in many places to the fabric itself. At the same time the crystals will be more or less surrounded by and mixed with the pyroxylin thereby forming a more or less intimate mixture between the pyroxylin and the ammonium phosphate, which mixture intimately unites with the fabric to 110

form a unitary structure. If the coating be physically separated from the fabric it will carry with it more or less of the ammonium phosphate. The essential functioning of the substances is that they cooperate to provide a fireproof for the fabric and a waterproof for the fireproof and the fabric, the composition also acting to shrink the fabric.

- 10 The fabric prepared in this way is effectively fireproof, also waterproof. By "waterproof," I mean not merely that quality which prevents the passage of water through the flexible material but that 15 quality by virtue of which the surface of the material remains intact, despite its continued contact with it, this latter quality resulting from the above described treatment. I believe that this action is due to 20 the fact that the crystals are submerged below the surface and are protected by the cellulosic composition. The tricresylphosphate materially reduces the inflammability of the pyroxylin so that the coating alone, 25 that is apart from the fabric, would have a low degree of inflammability. It may be called a coating of low or reduced inflammability. By applying this coating to the fireproofed fabric, such as that treated with 30 the ammonium phosphate, the resultant prepared fabric is thoroughly fireproof.

By suitably varying the process and the ingredients, a variety of so-called artificial leather may be prepared which, unlike many 35 artificial leathers, will be non-inflammable. Various other applications of the process will suggest themselves, such as for fireproofing sails and fabrics in various situations.

- 40 I have employed various proportions of the tricresylphosphate to the nitrocellulose, using in different cases all the way from 30 to 100 parts of the former to 100 parts of the latter. In general, the effect of increasing the amount of tricresylphosphate is to 45 decrease the shrinkage of the fabric and to increase the flexibility of the coating. The present application is a companion to my application, Serial No. 207,116, filed December 14, 1917, which application contains 50 generic claims to features not specifically claimed in the present application.

I claim:

- 55 1. The process of making a fireproof coated fabric, which consists in first impregnating the fabric with a solution of ammonium phosphate, drying out the solvent leaving the salt in the fabric, then applying one or more coats of a solution 60 containing pyroxylin and tricresylphosphate, and drying out the solvent after each coat, thereby shrinking the fabric and leaving a strong waterproof and fireproof fabric as the product.
- 65 2. The process of making a fireproof

coated fabric, which consists in first impregnating the fabric with ammonium phosphate, then drying the same, and then coating it with a composition containing pyroxylin.

70

3. The method of preparing a fireproof airplane wing with a fabric shrunken thereon, which consists in impregnating the fabric with a solution of an inorganic phosphate, and securing it loosely upon the wing frame, drying the fabric, and then coating it with a coating of pyroxylin and an aromatic phosphate and thereby shrinking it upon the frame.

75

4. The process of making a fireproof coated fabric, which consists in forming thereon in close association pyroxylin, an organic phosphate and an inorganic phosphate in sufficient quantity to effect noninflammability.

80

5. A fireproof coated fabric comprising a fabric carrying in close association, pyroxylin, an inorganic phosphate and an organic phosphate.

85

6. A fireproof coated fabric comprising a fabric carrying a fireproofing substance containing pyroxylin, ammonium phosphate and an aromatic phosphate.

90

7. A fireproof coated fabric comprising a fabric carrying in close association pyroxylin, ammonium phosphate and tricresylphosphate.

95

8. A product comprising a fabric coated with a composition containing a fireproofing substance adapted to give off water of combination in sufficient quantity to act effectively as a fire retarder, and pyroxylin.

100

9. A product comprising a fabric coated with a composition containing ammonium phosphate and pyroxylin.

105

10. A product comprising a fabric coated with a composition containing ammonium phosphate, pyroxylin and an inflammability reducer.

110

11. A waterproof body having on its surface pyroxylin and a fire retarding constituent adapted to give off a fire smothering gas containing ammonia.

115

12. A waterproof body having on its surface pyroxylin and a fire retarding constituent adapted to give off water of combination in sufficient quantity to act effectively as a fire retarder.

120

13. An article having on its surface a waterproof material comprising pyroxylin and ammonium phosphate.

125

14. A fireproof body adapted for use where a waterproof surface is required, said body having a surface material containing as a fire retarder ammonium phosphate and as a protector for the ammonium, pyroxylin.

130

15. A product containing in close association a compound of ammonia, pyroxylin and an aromatic phosphoric ester.

135

16. A product containing in close association a compound which will absorb heat and give off water upon decomposition, pyroxylin and an aromatic phosphoric ester. 5
17. A fabric carrying a pyroxylin composition which is adapted to dry to a fire-proof and waterproof material and which will shrink on drying and exert sufficient tensile strength to maintain its surface intact. 10
18. A product containing pyroxylin and a solvent therefor which lowers its inflammability and in close association therewith segregated fire extinguishing material. 15
19. A product consisting of a compound which will absorb heat and give off water upon decomposition, pyroxylin and tricresyl-phosphate in close association.
20. An article having a surface of tough, plastic material, composed of pyroxylin plasticized by an aromatic phosphate, the said material containing, as a fire retarding agent, ammonium phosphate.

WILLIAM G. LINDSAY.